

Sept. 9, 1941.

E. E. STAHL

**E. E. STAHLY**  
**POLYMERIZATION OF REFINERY UNSATURATES AND**  
**PREPARATION OF IMPROVED MOTOR FUELS**  
Filed Oct. 1, 1937

**2,255,275**



Eldon E. Stakly Inventor  
By P. J. Young Attorney

## UNITED STATES PATENT OFFICE

2,255,275

## POLYMERIZATION OF REFINERY UNSATURATES AND PREPARATION OF IMPROVED MOTOR FUELS

Eldon E. Stahly, Baton Rouge, La., assignor to Standard Oil Development Company, a corporation of Delaware

Application October 1, 1937, Serial No. 166,752

6 Claims. (Cl. 44—9)

The present invention resides in a method for producing gasoline hydrocarbons from normally gaseous hydrocarbons by acid polymerization of the latter. It is particularly directed to a process for converting mixtures of  $C_3$  and  $C_4$  olefins, with or without  $C_5$  olefins, by the action of sulfuric acid of suitable strength into liquid motor fuel. More particularly, it resides in a process in which normally gaseous mixed olefins of said type are converted into liquid fuel in a single operation.

It has already been proposed to subject hydrocarbon fractions containing mixtures of iso- and normal butylene with or without other unsaturated hydrocarbons to the action of sulfuric acid of a particular concentration at a temperature between about 150° F. and 300° F. to form  $C_8$  hydrocarbons composed of a mixture of di-iso-butylene and copolymer of normal and isobutylene. This mixture, either as such or preferably after hydrogenation, is a highly desirable constituent of a motor fuel.

A mixture of hydrocarbon polymers, mainly of branched chain structure ranging from  $C_8$  to  $C_{10}$  hydrocarbons and isopropyl ether and/or isopropyl alcohol, can be obtained by the method described above if the hydrocarbon fraction subjected to the acid treatment contains a mixture of  $C_3$ ,  $C_4$ , and  $C_5$  olefins. Such mixed polymers are preferably obtained in a single operation by subjecting a mixture of  $C_3$ ,  $C_4$ , and  $C_5$  olefins to the action of sulfuric acid of a concentration ranging from about 55% to about 80% at a temperature ranging from about 175° F. to about 300° F., and preferably under a pressure sufficient to maintain the normally gaseous hydrocarbons in the liquid state. When the feed stock is free from  $C_5$  hydrocarbons, the product will contain hydrocarbons ranging from  $C_8$  to  $C_{12+}$ .

The process may also be carried out in the gaseous phase. Due to the fact that the degree of dispersion of these hydrocarbons when in the gaseous phase in sulfuric acid is not as complete as when they are in the liquid phase, it is preferable, when carrying out the reaction in the

5 gaseous phase, to introduce the normally gaseous hydrocarbons into the reaction zone in the liquid state, the temperature in this zone being so correlated to the pressure that the hydrocarbons, upon being dispersed in the sulfuric acid, are converted to the gaseous phase.

The hydrocarbon polymers obtained by the above described methods are suitable for use as motor fuels, and have very pronounced anti-knocking characteristics. However, these polymers are unsaturated, and in many instances it is desirable to hydrogenate them in order to saturate the olefin double bonds before their use in gasoline. It has been found that this hydrogenation also reduces the alcohols and ethers present to the corresponding hydrocarbons, thereby causing a loss in the anti-knocking characteristics of such oxygenated compounds. An actual loss in yield of product suitable for use in gasoline also results, as isopropyl alcohol and ether are reduced to propane.

It has now been found that these losses can be prevented, and improved yields of improved motor fuels may be obtained by carrying out the process of the present invention. In one specific embodiment of the process the isopropyl ether formed is separated from the olefin polymer produced, the latter is hydrogenated wholly or in part, and the isopropyl ether is then reblended with the hydro-polymer and any residual olefin polymer. Other and further objects of this invention and illustrative embodiments thereof will be presented in the following description and in the attached drawing.

As previously stated, it is preferred, according to the present invention, to operate under a pressure such that the mixture of  $C_3$ ,  $C_4$ , and/or  $C_5$  hydrocarbons is maintained in the liquid state. At the preferred operating temperature of 200 to 225° F., a suitable pressure will be between 400 lbs./sq. in. and 600 lbs./sq. in. It is of course evident that the only upper limit on the pressure which may be employed is that dictated by economical operation. Under these preferred oper-

ating conditions the acid strength is preferably between 55% and 75%.

The effect of propylene on the product is noticeable when the feed stock contains even as little as 5 mole per cent of propylene based on a total feed containing 48.5 mole per cent of olefins. Generally it will be desirable to employ a feed having a higher percentage of propylene. Preferably, it should be present in an amount at least equal to the amount of butylenes where these are the only olefins in the feed stock. An increase in the ratio of propylene to normal butylene over one to one favors the formation of isopropyl ether. In general, it may be stated that any feed stock which contains a substantial amount of propylene, together with C<sub>4</sub> and/or C<sub>5</sub> olefins, is suitable for the process of the present invention.

The feed stock most commonly employed for the process of the present invention is a refinery gas obtained from crude distillation, cracking, destructive hydrogenation, or other thermal process. These gases may contain as high as 50% of olefins composed mainly of propylene, iso- and normal butylene with small amounts of the amylenes. The remainder of such refinery gases consists of C<sub>1</sub> to C<sub>5</sub> paraffins and hydrogen. The capacity of the polymerization chamber may be increased by isolating the olefinic constituents from the refinery gas by any suitable method, such as by liquefaction of the C<sub>3</sub> to C<sub>5</sub> constituents of such gases and the extraction of the olefins from said liquefied fraction by any common selective solvent such as sulfur dioxide. Or, if desired, the C<sub>3</sub> to C<sub>5</sub> hydrocarbons may be segregated from the lighter constituents.

When the only available feed stock is one mainly composed of C<sub>3</sub> and C<sub>4</sub> paraffins with or without C<sub>5</sub> paraffins, it is necessary to subject it to a thermal treatment for the conversion of the paraffins to olefins. This conversion may be either cracking or catalytic dehydrogenation, preferably the latter. A particularly suitable feed stock is one obtained by the cracking or catalytic dehydrogenation of a mixture of propane and isobutane or a naturally occurring mixture of iso- and normal butane with propane. The former, when thermally decomposed, produces an olefinic mixture mainly composed of propylene and isobutylene which, when subjected to the process of the present invention, yields a mixture of olefins of particularly highly branched nature, together with isopropyl ether. This mixture, especially when the olefinic constituents thereof are hydrogenated, is an exceptionally good blending agent for motor fuels.

The reaction time best suited for the process of the present invention may be most readily understood when expressed in liters of liquid hydrocarbon feed per hour per foot of acid height in the polymerization zone. This feed rate may vary between about 1½ liters per hour per foot of acid height and about 7 liters per hour per foot of acid height with an acid column having a cross sectional area of about 0.05 sq. ft. These specific values are only exemplary, since they will vary with acid columns of different cross-sectional area. They are, however, indicative of the order of feed rate to be employed and can be readily ascertained for each individual case. The liquid hydrocarbon feed may be introduced into the acid in the polymerization zone thru a porous thimble, such as an alundum thimble, or thru jets which impart a high degree of dispersion to the liquid feed. Sat-

isfactory results have been obtained with jets having openings of 0.018" and 0.023". It is, of course, apparent that the size of the jet opening may be chosen to suit different total feed rates.

After the separation of the normally liquid constituents from the product issuing from the polymerization zone, a residual gas mixture, which still contains a substantial percentage of C<sub>3</sub> to C<sub>5</sub> olefins, may be obtained. This residual gas mixture may be recycled to the fresh feed, or may be sent thru a second polymerization unit of the same type. When recycling is employed, saturated normally gaseous hydrocarbons build up in the feed. For this reason, it is advantageous from time to time to divert the recycled stock to a cracking or catalytic dehydrogenation chamber wherein the saturates are converted to corresponding olefins. Alternatively, the recycle gas may be diverted to a thermal polymerization unit for the conversion of normally gaseous paraffins into hydrocarbons boiling within the gasoline range.

When catalytic dehydrogenation is employed, the dehydrogenation chamber is maintained at a temperature ranging from about 950 to 1100° F. and under atmospheric or only slightly elevated pressure. A suitable catalyst for this conversion is one containing, as its essential catalytic constituent, an oxide or a sulfide, or other compound, of a metal of group VI of the periodic system which is preferably associated with a carrier, such as bauxite, kaolin, alundum, active carbon, etc., or with a difficultly reducible oxide, such as alumina, thoria, silica, etc. When a thermal polymerization unit is employed for processing the recycle gas, it is maintained under a pressure of at least 500 lbs./sq. in. and under a temperature between about 900° F. and 1200° F., depending upon the composition of the recycle gas.

Ordinarily the acid in the polymerization zone passes therethru concurrent with the hydrocarbon feed and the mixture of acid, unconverted feed and product is discharged into a separator in which the acid settles to the bottom from which it is drawn off and returned to the reaction chamber. During the process a content of alkyl sulfates, mainly isopropyl sulfate, is built up in the acid. Up to a certain extent the presence of these sulfates in the acid exerts a beneficial effect upon the equilibrium of the polymerization process. For this reason it may be desirable to add alkyl sulfates to the fresh feed.

Should the content of alkyl sulfates in the circulating acid become so high that removal of some or all of these sulfates is desirable, this may be done by arranging in the acid return line a reaction chamber maintained under conditions suitable for the decomposition of these alkyl sulfates. This chamber may be so operated, namely, at a temperature somewhat above the temperature employed in the main reaction zone, as to convert the alkyl sulfates into ethers containing small amounts of alcohols. Alternatively a hydrolyzing agent, such as water or an alkali, may be fed into this chamber and the conditions so adjusted in a known manner as to convert the alkyl sulfates into the corresponding alcohols containing small amounts of ether. When this latter method is employed, it is usually necessary to adjust the concentration of the acid before reintroducing it into the polymerization zone. If caustic soda is used as the hydrolyzing agent, it is unnecessary to take measures to remove the resulting sodium acid sulfate or sodium sulfate

from the circulating acid, since the presence of either of these salts is not detrimental to the polymerizing action of the sulfuric acid.

As previously stated, it is preferable to hydrogenate at least part of the normally liquid olefinic hydrocarbons obtained as a result of the acid treatment. If these liquid products are free from sulfur, the hydrogenation is preferably carried out in the presence of a highly active nickel catalyst, that is a nickel catalyst prepared by the roasting and reduction with hydrogen of a freshly precipitated nickel compound. The nickel so prepared is used to best advantage when disposed on a carrier, such as kaolin, pumice, etc. When such a catalyst is employed, the hydrogenation is generally carried out at a pressure of at least 50 lbs./sq. in. and at a temperature between about 300° and 600° F.

Should the normally liquid hydrocarbon product contain sulfur, it is advisable to employ a hydrogenating catalyst which is immune to poisoning by sulfur. The preferred catalysts of this type are those which have previously been mentioned for use in the dehydrogenation of normally gaseous hydrocarbons. When a catalyst of this type is employed, the temperature best suited for the hydrogenation is generally somewhat higher than that required for hydrogenation in the presence of a nickel catalyst.

If it is desired to employ a nickel catalyst for the hydrogenation operation, measures may be taken to preclude the presence of sulfur in the liquid hydrocarbon feed to the hydrogenation chamber. This is best accomplished by scrubbing the normally gaseous hydrocarbons employed as a feed stock to the polymerization chamber with caustic. The elimination of sulfur from this feed stock also improves the polymerization stage of the process. Sulfur may often be removed from the normally liquid products by suitable fractionation. The content of sulfur in these products may also be reduced to the necessary extent by caustic washing or by treatment of these products in the vapor phase with a desulfurizing agent, such as bauxite, ferrous sulfide, fuller's earth, alumina and the like.

While in the preferred embodiment of the present invention the isopropyl ether is separated from the normally liquid product before the latter is subjected to hydrogenation, this step may be modified. The separated isopropyl ether will always contain a considerable amount of hexylene which is formed in the polymerization chamber and which may be improved as a motor fuel constituent by hydrogenation. The complete separation of these two compounds by fractionation is practically impossible, and it may accordingly be desirable in producing a highly saturated motor fuel to remove, prior to the hydrogenation, only so much of the isopropyl ether as can be separated substantially free of hexylene.

This separation of the isopropyl ether from the hydrocarbon polymers may also of course be carried out in any other suitable manner, such as by treatment of the reaction product with solvents having a selective solvent action between the ether and the hydrocarbons, such as aqueous alcohol.

The products of the process of the present invention, having a highly branched structure and having a boiling range nearly commensurate with that of gasoline, can be readily converted into a gasoline of high octane number by the addition of the necessary amount of low boiling hydrocarbons to properly adjust their vapor pressure,

and the addition, if necessary, of certain high boiling compounds to provide a gasoline of the necessary end point. As suitable additions of low boiling point may be mentioned iso-pentane and butane or iso-butane. When it is necessary to add high boiling hydrocarbons this may be done with a simultaneous improvement in the octane number of the total blend by the addition of aromatic extracts of heavy naphthas, that portion of the extract which has an end boiling point of about 400° F. being selected. In many instances, however, the product of the process of the present invention has a sufficiently high end point to make the addition of extraneous heavy hydrocarbons unnecessary.

The nature of the process of the present invention is graphically illustrated in the accompanying drawing in which the single figure is a front elevation in diagrammatic form of an apparatus suitable for carrying out said process.

Referring to the drawing in detail, 1 is a feed line for the introduction of C<sub>3</sub> to C<sub>5</sub> hydrocarbons into the unit. Arranged in line 1 is a compressor 2 by which the C<sub>3</sub> and C<sub>5</sub> hydrocarbons are liquefied and pumped thru the system. The liquefied feed stock is fed into polymerization chamber 3 through a porous thimble 4. Sulfuric acid of suitable strength is fed into chamber 3 at its bottom through line 5.

The mixture of sulfuric acid, unconverted feed and reaction product leaves reaction chamber 3 through line 6, passes through cooler 7 into a settling chamber 8 provided with an interface indicator 9. The sulfuric acid settles to the bottom and is drawn off through line 5, which returns it to the reaction chamber 3. The mixture of normally liquid reaction product and liquefied normally gaseous unconverted feed leaves separator 8 through line 10, which discharges it into still 11 which is maintained under such conditions that unconverted feed, isopropyl ether, and any hexylene formed, leaves the top thereof in vapor form through line 12, and hydrocarbons having seven or more carbon atoms leave the bottom in the liquid state through line 13 which is provided with a valve 14 and a branched line 15 in which the flow of liquid is controlled by valve 16. With valve 16 closed and valve 14 open, the liquid reaction product is conducted by line 13 to storage tank 17. By suitably controlling valves 14 and 16, part or all of the liquid product may be conducted by line 15 through heating coil 18 into hydrogenation chamber 19.

Line 15 is provided with a branch 20 through which the necessary hydrogen for the hydrogenation of the liquid product is introduced into the hydrogenation chamber. The product from the hydrogenation chamber passes into separator 21 from which the hydrogenated hydrocarbons are drawn off at the bottom through line 22 by which they are fed to storage tank 23. Excess hydrogen leaves separator 21 through line 24 and may be recycled to the hydrogenation chamber.

The unconverted feed and the products boiling below C<sub>7</sub> hydrocarbons are conducted by line 12 to a partial condenser 25 in which part of the higher boiling constituents thereof are liquefied and returned to the top of still 11 as reflux condensate by line 26. The remainder of the mixture leaves condenser 25 through line 27 by which it is fed to cooling coil 28 after the pressure thereon has been sufficiently released by pressure release valve 29 in line 27. The mixture is then discharged into a separating chamber 30 provided with a liquid level indicator. Isopropyl

ether and any C<sub>6</sub> hydrocarbons present are drawn off from the bottom of separator 30 by line 31 and fed into a storage tank 32.

The residual C<sub>3</sub> to C<sub>5</sub> hydrocarbons leave the top of separator 30 by line 33 after which they are compressed in compressor 33a and returned through line 33b to reaction chamber 3.

Line 33 is provided with a valve 34 and, at a point just ahead of this valve, with a branch line 35 controlled by valve 36. Arranged in the branch line 35 is a reaction chamber 37 which, as previously stated, may be employed for cracking, catalytic dehydrogenation or thermal polymerization. When this vessel is employed for cracking or catalytic dehydrogenation, the effluent therefrom passes through line 38 to a separator 39 from the top of which C<sub>2</sub> and lighter hydrocarbons are removed from the system and from the bottom of which C<sub>3</sub> to C<sub>5</sub> hydrocarbons are pumped through line 40 to line 33b.

Line 38 is provided with a valve 41 and with a branch line 42 controlled by a valve 43. When chamber 37 is employed for thermal polymerization, valve 41 is closed and valve 43 is opened, and the effluent from said chamber passes through branch line 42 into separator 44 from which gasoline and heavier hydrocarbons are withdrawn by line 46, and C<sub>5</sub> and lighter hydrocarbons pass overhead through line 47 back to line 38.

Line 5 is provided with a valve 48 and a branch line 49 controlled by a valve 50. When it is desired to remove alkyl sulfates from the circulating sulfuric acid, valve 48 is closed, valve 50 is opened, and the acid, containing alkyl sulfates, removed from separator 8, is introduced into a chamber 51 which may be operated as a hydrolyzing zone, in which event a hydrolyzing agent is introduced thereto through inlet 52, or as a reaction chamber for the production of ethers. The alcohol or ether, as the case may be, leaves vessel 51 through line 53 in which it is conducted to cooler 54 and thence to storage chamber 55. Sulfuric acid, which may contain the water added for hydrolysis, leaves vessel 51 through line 56, goes to a concentrator 57, which may be heated in any suitable manner, and then through line 58 back to line 5. Line 58 is provided with an inlet 59 for fresh acid.

Tanks 17, 23, 32, and 55 are provided respectively with outlets 60, 61, 62, and 63 leading to a common line 64. This arrangement facilitates the blending of the products contained in the various storage tanks in any desired proportions.

It is apparent that many changes may be made in the above described apparatus without departing from the scope of the present invention. A number of the possible modifications have already been indicated. A showing of various conventional expedients, such as means for cooling the hydrogenation chamber 19, a liquefaction and compression apparatus in line 33, and heat exchange devices at various appropriate points, has been purposely omitted in the interest of simplicity. The following experimental data are offered to illustrate the effect of changes in operating conditions and acid concentration on the nature of the product.

Six runs were made with a three-foot height of sulfuric acid with a cross-sectional area of 4.9 sq. in. under a pressure of 600 lbs./sq. in. The feed was introduced into the acid through a jet having an internal diameter of 0.018". One of the runs was made at 266° F. in the gas phase to determine what effect a change of phase would have on the yield. Since jet dispersion of gases

is not as efficient as that of liquids, the feed in this run was not preheated whereby it was dispersed as liquid and converted to gas in the reactor. The data for these runs may be summarized as follows:

|                                                        | Run No. |      |      |      |      |      |
|--------------------------------------------------------|---------|------|------|------|------|------|
|                                                        | 1       | 2    | 3    | 4    | 5    | 6    |
| Feed rate, l./hr.                                      | 15      | 16   | 15   | 15   | 15   | 13   |
| Weight percent acid                                    | 50      | 60   | 69   | 69   | 69   | 66   |
| Temperature, ° F.                                      | 224     | 215  | 224  | 221  | 206  | 200  |
| Feed:                                                  |         |      |      |      |      |      |
| Mole percent ethane                                    | 0.6     | 0.6  | 0.6  | 0.8  | 0.8  | 0.1  |
| Mole percent propylene                                 | 12.5    | 12.5 | 12.5 | 12.8 | 12.8 | 12.1 |
| Mole percent propane                                   | 56.1    | 56.1 | 56.1 | 53.1 | 53.1 | 66.3 |
| Mole percent isobutylene                               | 3.4     | 3.4  | 3.4  | 3.7  | 3.7  | 2.2  |
| Mole percent n-butlenes                                | 7.1     | 7.1  | 7.1  | 7.0  | 7.0  | 4.1  |
| Mole percent butanes                                   | 20.1    | 20.1 | 20.1 | 22.2 | 22.2 | 14.9 |
| Mole percent C <sub>5</sub> +                          | 0.2     | 0.2  | 0.2  | 0.4  | 0.4  | 0.3  |
| Exit gas:                                              |         |      |      |      |      |      |
| Mole percent ethane and lighter                        | 3.6     |      | 1.8  | 1.8  |      | 0.2  |
| Mole percent propylene                                 | 11.0    |      | 6.9  | 6.8  |      | 7.2  |
| Mole percent propane                                   | 55.4    |      | 60.6 | 60.3 |      | 68.6 |
| Mole percent isobutylene                               | 2.7     |      | 0.4  | 0.8  | 0.6  | 0.6  |
| Mole percent n-butylene                                | 6.0     |      | 4.9  | 5.0  |      | 3.1  |
| Mole percent butanes                                   | 20.8    |      | 25.1 | 25.0 |      | 18.3 |
| Mole percent C <sub>5</sub> +                          | 0.5     |      | 0.3  | 0.3  |      | 2.0  |
| 20 Yield on propylene:                                 |         |      |      |      |      |      |
| Based on product                                       | 12.0    | 41   | 65   | 54   | 65   |      |
| Based on olefin reduction                              | 16.0    |      | 94   | 90   | 86   | 75   |
| Yield on total unsats.:                                |         |      |      |      |      |      |
| Based on product                                       | 19.3    |      | 31   | 27   | 32   |      |
| Based on olefin reduction                              | 17.5    |      | 52   | 50   | 48   | 45.5 |
| Olefin reductions:                                     |         |      |      |      |      |      |
| Percent reduction of iso C <sub>4</sub> H <sub>8</sub> | 23      |      | 91   | 94   | 87   | 75   |
| Percent reduction of n-C <sub>4</sub> H <sub>8</sub>   | 18      |      | 39   | 34   |      | 30   |
| Percent reduction of propylene                         | 16.0    |      | 51   | 52   |      | 43   |
| Percent reduction of total unsats.                     | 17.5    |      | 52   | 50   | 48   | 45.5 |
| Product:                                               |         |      |      |      |      |      |
| I. B. P., ° F.                                         | 129     | 97   | 98   | 93   | 116  | 123  |
| 5%                                                     | 171     | 150  | 147  | 144  | 174  | 163  |
| 80%                                                    | 183     | 303  | 309  | 333  | 356  | 284  |
| F. B. P., ° F.                                         | 226     | 410  | 341  | 362  | 442  | 336  |
| Percent recovery                                       | 99.0    | 90.0 | 91.0 | 89.0 | 94   | 98.5 |

It will be noted that with 50% acid the yield was mainly isopropyl alcohol. This is evident from the fact that whereas only 5% of the product distilled over at 171, 80% distilled over at 183. It is also to be observed that the gas phase experiment gave a yield comparable to that obtained with the same feed rate and acid strength in liquid phase at a temperature of 224° F. The product of the gas phase operation, however, was somewhat higher boiling, indicating the presence of higher polymers.

The products of the runs made with acid of higher than 50% concentration contained varying amounts of isopropyl ether ranging from about 5% to 10%. The amount of isopropyl alcohol in the various products, not taking into consideration the isopropyl alcohol recovered from the circulating acid, ranged from about 1% to 3%.

The products from Runs 3 and 4 were mixed and distilled to 329° F.; 75% of the mixture was recovered as overhead. This overhead was hydrogenated in the presence of nickel at 500° F. under a pressure of 1600 lbs./sq. in. A 40% blend of the hydrogenated product in a 74 octane number straight-run naphtha gave a blending octane number of 93. A similar blend of the straight-run naphtha with iso-octane indicated the blending octane number of the iso-octane to be 92.5. Thus the hydrogenated product of the acid treatment of the C<sub>3</sub> and C<sub>4</sub> cut is about equal to iso-octane as a blending agent for octane number improvement.

Spent acid from Run No. 3 was diluted with water and subjected to distillation. The product

of the distillation was a 70% aqueous solution of isopropyl alcohol. In the run itself 1616 grams of liquid product was obtained. 1000 grams of isopropyl alcohol was obtained from the spent acid. Thus, the total weight per cent yield of product, based on the propylene, was 65% (shown in the data above) plus 28.6% (yield of alcohol) or 93.6%. This figure checks with the figure given in the above table for yield based on propylene reduction.

Several analytical distillations were run on products of polymerization of propane-butane mixtures. The estimates of the compositions of the various products are tabulated below with the respective feeds to the polymerization unit for the several products.

normal butylene. The results were as follows:

|                                     |      | Run No. |   |
|-------------------------------------|------|---------|---|
|                                     |      | 7       | 8 |
| Polymer yields:                     |      |         |   |
| Volume percent on feed              | 22.3 | 9.9     |   |
| Weight percent on total unsaturates | 62.5 | 55.1    |   |
| Weight percent on isobutylene       | 173  | 191     |   |
| Polymerization:                     |      |         |   |
| Percent propylene polymerized       | 58.5 |         |   |
| Percent isobutylene polymerized     | 97.9 | 96.5    |   |
| Percent normal butylene polymerized | 40.4 | 38.4    |   |
| Polymer inspections:                |      |         |   |
| Percent at 300° F.                  | 82   | 85      |   |
| Octane No. of 85% O. H. ASTM        | 85.2 | 84.3    |   |
| Octane No. of hydro total polymer   | 94.4 | 95.5    |   |

The product obtained in Run No. 7 over a reac-

|                                                                                                          | Sample No.  |             |             |           |            |
|----------------------------------------------------------------------------------------------------------|-------------|-------------|-------------|-----------|------------|
|                                                                                                          | 1           | 2           | 3           | 4         | 5          |
| Temp., °F.                                                                                               | 225         | 225         | 224         | 221       | 200        |
| Weight percent acid                                                                                      | 69          | 69          | 69          | 69        | 66         |
| Acid height, feet                                                                                        | 3           | 3           | 3           | 3         | 3          |
| Feed:                                                                                                    |             |             |             |           |            |
| Mole percent <i>t</i> -C <sub>4</sub> H <sub>8</sub>                                                     | 3.1         | 5.4         | 3.4         | 3.7       | 2.2        |
| Mole percent <i>n</i> -C <sub>4</sub> H <sub>8</sub>                                                     | 7.9         | 9.7         | 7.1         | 7.0       | 4.1        |
| Mole percent C <sub>3</sub> H <sub>8</sub>                                                               | 8.6         | 7.5         | 12.5        | 12.8      | 12.1       |
| Total                                                                                                    | 19.6        | 22.6        | 23.0        | 23.5      | 18.4       |
| Ratio: Iso-C <sub>4</sub> H <sub>8</sub> /n-C <sub>4</sub> H <sub>8</sub> /C <sub>3</sub> H <sub>8</sub> | 1/2.5/2.8   | 1/1.8/1.4   | 1/2.1/3.7   | 1/1.9/3.5 | 1/1.86/5.5 |
| Percent reacted:                                                                                         |             |             |             |           |            |
| <i>t</i> -C <sub>4</sub> H <sub>8</sub>                                                                  | 87          | 87          | 91          | 94        | 75         |
| <i>n</i> -C <sub>4</sub> H <sub>8</sub>                                                                  | 33          | 29          | 39          | 34        | 30         |
| C <sub>3</sub> H <sub>8</sub>                                                                            | 43          | 40          | 51          | 52        | 45         |
| Ratio of olefins reacted:                                                                                |             |             |             |           |            |
| C <sub>4</sub> H <sub>8</sub> /n-C <sub>4</sub> H <sub>8</sub>                                           | 1.42/1      | 1.07/1      | 2.36/1      | 2.8/1     | 4.4/1      |
| Iso-C <sub>4</sub> H <sub>8</sub> /n-C <sub>4</sub> H <sub>8</sub> /C <sub>3</sub> H <sub>8</sub>        | 1.04/1/1.42 | 1.68/1/1.07 | 1.15/1/2.37 | 1.5/1/2.8 | 1.32/1/4.4 |
| Iso-C <sub>4</sub> H <sub>8</sub> /other olefins                                                         | 1/2.33      | 1/1.23      | 1/2.9       | 1/2.6     | 1/4.1      |
| Percent reduction of unsats.                                                                             | 46          | 46.5        | 52          | 50        | 45.5       |
| Estimates of product:                                                                                    |             |             |             |           |            |
| Percent isopropyl ether                                                                                  | 8           | 5           | 10          |           | 10         |
| Percent C <sub>4</sub> +C <sub>5</sub> hydrocarbons                                                      | 14          | 14          | 11          |           | 15         |
| Percent C <sub>6</sub> hydrocarbons                                                                      | 62          | 52          | 38          |           | 25         |
| Percent C <sub>7</sub> -C <sub>12</sub> +hydrocarbons                                                    | 13          | 23          | 38          |           | 46         |
| Percent loss                                                                                             | 3           | 6           | 3           |           | 4          |
|                                                                                                          | 100.0       | 100.0       | 100.0       |           | 100.0      |

The per cent isopropyl ether in the product apparently increases with increasing feed ratio of C<sub>3</sub>H<sub>8</sub> to C<sub>4</sub>H<sub>8</sub>. Samples 5 and 3 contain a considerably higher percentage of material above C<sub>8</sub> hydrocarbons than found in Samples 1 and 2. This indicates that higher C<sub>3</sub>H<sub>8</sub>/C<sub>4</sub>H<sub>8</sub> feed ratios tend to increase the amount of higher boiling polymers (C<sub>9</sub>-C<sub>12</sub>+hydrocarbons).

Samples 3 and 4 had the following boiling characteristics:

|                  | Sample 3 | Sample 4 |
|------------------|----------|----------|
| I. B. P.         | 92       | 96       |
| 5%               | 128      | 146      |
| 20%              | 198      | 212      |
| 80%              | 309      | 333      |
| F. B. P.         | 338      | 346      |
| Percent recovery | 88.0     | 87.0     |

Comparative results, obtained by processing a feed containing propylene and butylenes and one containing only butylenes respectively, were obtained by treating the respective feeds in a reaction chamber having an 11 ft. height of 60% sulfuric acid with a cross-sectional area of 9.6 sq. in. The operating temperature was 225° F., the pressure was 425 lbs./sq. in. and the feed rate was 24 liters/hour. The feed was introduced into the reaction chamber through a jet having an internal diameter of 0.023".

In Run No. 7 the feed contained 4.9% propylene, 17.1% isobutylene, and 26.5% of normal butylene. In Run No. 8 the feed contained no propylene, 7.2% of isobutylene, and 18.4% of

the reaction period of 132 hours had the following average characteristics:

|                     |      |  |
|---------------------|------|--|
| 45 Product:         |      |  |
| ° A. P. I. gravity  | 56.7 |  |
| I. B. P., ° F.      | 129  |  |
| 5%                  | 196  |  |
| 10%                 | 210  |  |
| 20%                 | 221  |  |
| 30%                 | 226  |  |
| 40%                 | 231  |  |
| 50%                 | 235  |  |
| 60%                 | 243  |  |
| 70%                 | 253  |  |
| 80%                 | 283  |  |
| 90%                 | 350  |  |
| 95%                 | 359  |  |
| F. B. P., ° F.      | 361  |  |
| Recovery            | 97.5 |  |
| Residue             | 1.3  |  |
| Aniline point, ° F. | 103  |  |

An analytical distillation of this product showed that, on the average, it contained about 2% of isopropyl ether. A cut of this product obtained by distilling the product to an 85% overhead yielded, upon hydrogenation, a product having an octane number of 95.6. The unhydrogenated product usually contains about 9 and 10 mole per cent reacted propylene in the form of ether, alcohol, and the unsaturated hydrocarbons C<sub>6</sub>H<sub>12</sub>, C<sub>7</sub>H<sub>14</sub>, and C<sub>8</sub>H<sub>16</sub>, and higher hydrocarbons. The first fraction from the distillation of this product has an ethereal odor. The presence of hexylene

in this first overhead was indicated by its refractive index and boiling point.

The following example illustrates advantages of operation according to the preferred method of this invention. A crude polymer, obtained by co-polymerization of C<sub>3</sub> and C<sub>4</sub> olefins and containing isopropyl ether, was found to have an octane number of 85.6. Hydrogenation of this polymer product to saturate the double bonds produces a saturated product having an octane number of 90.0. But when the isopropyl ether is separated before the hydrogenation, the remaining polymer being hydrogenated under the same conditions as before, and the isopropyl ether is then reblended with the hydrogenated polymer, the final blend has an octane number of 93.3. In addition to this increased octane number, the yield is also greater in the second case as hydrogenation of isopropyl ether to propane is avoided.

The experiments described above do not, of course, define the metes and bounds of the present invention. They are complete operations carried out under various conditions falling within the broad ranges of operating conditions heretofore described and established by experiments of a qualitative nature.

It is to be understood that while it is preferred to employ, as a feed stock in the process of the present invention, one containing propylene and both iso- and normal butylene, this process may be practiced successfully on any feed stock containing propylene and any olefin containing 4 or 5 carbon atoms.

The nature and objects of the present invention having been thus described and illustrated, what is claimed as new and useful, and desired to be secured by Letters Patent is:

1. A process for the production of a motor fuel of high octane number which comprises contacting a mixture the olefin content essentially comprising propylene and at least one other olefin of higher molecular weight and having no hydrocarbon constituents containing more than 5 carbon atoms with sulfuric acid of a concentration between 55% and 75% at a temperature between 175° and 300° F. and under elevated pressure, separating a reaction product predominantly boiling within the gasoline range and containing a minor amount of isopropyl ether from the sulfuric acid, dividing the reaction product into a fraction containing isopropyl ether and a hydrocarbon fraction boiling in the motor fuel range, then saturating the double bonds in the said hydrocarbon fraction with hydrogen.

2. A process for the production of a motor fuel of high octane number containing isopropyl ether which comprises contacting a mixture the olefin content essentially comprising propylene and at least one other olefin of higher molecular weight

containing less than 6 carbon atoms with sulfuric acid under conditions causing the formation of a polymerization reaction product predominantly containing hydrocarbon polymers boiling in the motor fuel range and a minor amount of isopropyl ether, removing the reaction product from the sulfuric acid, dividing the reaction product into a fraction containing isopropyl ether and a hydrocarbon fraction, saturating the double bonds in the said hydrocarbon fraction with hydrogen, and combining the hydrogenated product with the fraction containing isopropyl ether.

3. A process for the production of a motor fuel of high octane number containing isopropyl ether which comprises contacting a mixture the olefin content essentially comprising propylene and at least one other olefin of higher molecular weight and having no hydrocarbon constituents containing more than 5 carbon atoms with sulfuric acid of a concentration between 55% and 75% at a temperature between 175° and 300° F. and under elevated pressure, removing the reaction product and unconverted initial material from the sulfuric acid, separating the reaction product from the unconverted initial material, dividing the reaction product into a fraction containing isopropyl ether and a higher boiling hydrocarbon fraction, said latter fraction constituting the major portion of the reaction product, saturating the double bonds in the said higher boiling hydrocarbon fraction with hydrogen, and combining the hydrogenated product with the fraction containing isopropyl ether.

4. A process according to claim 3 in which the feed stock is a mixture containing C<sub>3</sub> and C<sub>4</sub> olefins.

5. A process according to claim 3 in which the said mixture is passed through a body of sulfuric acid at a rate varying between about 1½ and 7 liters/hr./ft. of acid height of a cross-sectional area of about 0.05 sq. ft.

6. In the process for the production of motor fuel of high octane number by contacting a hydrocarbon mixture, the olefin content of which essentially comprises propylene and at least one olefin of higher molecular weight containing less than six carbon atoms per molecule, with sulfuric acid under conditions causing the formation of a polymerization reaction product predominantly containing hydrocarbon polymers boiling in the motor fuel range and a minor amount of isopropyl ether, and removing the reaction product from the sulfuric acid mixture, the improved steps comprising separating a fraction containing substantially all of the isopropyl ether from the reaction product and hydrogenating at least a portion of the substantially isopropyl-ether-free reaction product.

ELDON E. STAHLY.